

# United States Patent

[11] 3,617,290

[72] Inventor **Henry Walter Wood**  
**Ilford, England**

[21] Appl. No. **702,543**

[22] Filed **Feb. 2, 1968**

[45] Patented **Nov. 2, 1971**

[73] Assignee **Ilford Limited**  
**Ilford, England**

[32] Priority **Feb. 13, 1967**

[33] **Great Britain**

[31] **6,830/67**

2,716,062 8/1955 Carroll et al. .... 96/109 X  
3,155,506 11/1964 Blake ..... 96/107 X

*Primary Examiner—Norman G. Torchin*

*Assistant Examiner—Won H. Louie, Jr.*

*Attorney—Cushman, Darby and Cushman*

[54] **BARBITURIC ACID DERIVATIVES STABILIZERS  
FOR EMULSIONS SENSITIZED WITH ETHYLENE  
OXIDE CONDENSATE**  
**6 Claims, No Drawings**

[52] U.S. Cl. .... **96/94,**

**96/107, 96/109**

[51] Int. Cl. .... **G03c 1/02**

[50] Field of Search. .... **96/94, 109,  
107**

[56] **References Cited**

UNITED STATES PATENTS

1,025,872 5/1912 Hoerlein ..... 260/257

**ABSTRACT:** This application describes a process for the production of a gelatino silver halide emulsion which comprises forming the emulsion by a technique including a step wherein the emulsion is sulfur sensitized, and adding to the emulsion (1) an ethylene oxide condensate in quantity sufficient to increase the speed of the emulsion and the contrast of images developed therein, and (2) at least 1 g. per gram mole of silver halide present, of a compound of the general formula:



wherein R<sub>1</sub> is an aryl group and R<sub>2</sub> is a lower alkyl group.

**BARBITURIC ACID DERIVATIVES STABILIZERS FOR  
EMULSIONS SENSITIZED WITH ETHYLENE OXIDE  
CONDENSATE**

This invention relates to photographic materials and more particularly to the production of photographic gelatino silver halide emulsions. It is of particular significance in the production of emulsions designed to record X-radiation and will be described with particular reference thereto.

It is known that the sensitivity of a photographic gelatino silver halide emulsion may be increased by the addition to the emulsion of a nonionic wetting agent which is an ethylene oxide condensate or polyethylene oxide derivative. Besides modifying the physical character of coated layers of such emulsions the ethylene oxide compounds increase both the speed of the emulsions and the contrast of the developed images, and this may be due to acceleration of development.

When such ethylene oxide compounds are added to emulsions of the type generally prepared for use in X-radiography, these advantages are to some extent obtained, but the tendency of such additives to increase the fog density of the emulsion, especially after incubation, is found to be severe.

Various attempts have been made to reduce the fog level which arises from the use of ethylene oxide compounds by the addition of so-called antifogging agents. The bulk of those tested, however, have been found to be insufficiently effective.

It is the object of the present invention to provide a process for the production of silver halide emulsions so sensitized in which the fog level on development is reduced.

According to the present invention there is provided a process for the production of a gelatino silver halide emulsion which comprises forming the emulsion by a technique including a step wherein the emulsion is sulfur sensitized, and adding to the emulsion (1) an ethylene oxide condensate in quantity sufficient to increase the speed of the emulsion and the contrast of images developed therein, and (2) at least 1 g. per gram mole of silver halide present, of a compound of the general formula I<sub>2</sub>—



wherein R<sub>1</sub> is an aryl group and R<sub>2</sub> is a lower alkyl group.

By lower alkyl is meant an alkyl group containing up to six carbon atoms.

The preferred compound of formula I is phenobarbitone wherein R<sub>1</sub> is phenyl and R<sub>2</sub> is ethyl.

The compounds are preferably added to the emulsion as aqueous solutions, to which end an equivalent of an alkali hydroxide is used. Alternatively, the compounds may be used in the form of their soluble sodium salts. Optionally, an equivalent of an acid, such as HCl may also be added to maintain the pH of the emulsion at its original level.

Any of the ethylene oxide condensates and derivatives known from the literature to have a sensitizing effect on photographic silver halide emulsions may be employed. Preferred compounds are ethylene oxide homopolymers which are marketed under the trade name Carbowax and having relatively high molecular weights, e.g. 4,000 or more. However, derivatives such as the aromatic and alkyl ethers thereof, e.g. the commercial product Texofor F.60, are also of especial value. (The word Texofor is a Registered Trade Mark).

The quantity used will, of course, vary with the effect desired, but generally may be up to 20 grams of the condensate per gram mole of silver halide in the emulsion, e.g. 1 to 20 grams.

The quantity of the additive of the general formula given above will also vary with the circumstances, but will be at least 1 gram per gram mole of silver halide in the emulsion, and optionally substantially larger, e.g. up to 255 grams per gram mole of silver halide, or even more.

The ethylene oxide condensate and the compound of the

general formula given above may be added to the emulsion at any convenient stage in the manufacture of the emulsion but they are preferably added at the stage after the digestion of the emulsion.

It is believed that the additives act by forming weak complexes with the polyethylene oxides, which does not, however, prevent the latter from exercising their sensitizing function.

The following example will serve to illustrate the invention and the improvement in results which can be obtained by use of the invention.

**EXAMPLE**

A gelatino silver iodobromide emulsion was prepared in a manner conventional for emulsions to be used for X-radiography. The emulsion which was not color sensitized, contained 200 g. of gelatin per gram mol of silver halide and was sensitized by means of sulfur compounds and gold salts in manner known per se. The emulsion was divided into three parts:

- 20 1. No further addition was made.
- 20 2. Polyethylene oxide of molecular weight 6000 was added at the rate of 2 g. per gram mol of silver halide.
- 20 3. The same addition was made as for (2), and in addition there was added 10 g. of the sodium salt of the phenobarbitone per gram mole of silver halide, and an equivalent amount of hydrochloric acid.

The three emulsions were coated on film and exposed. They were then developed in a Phenidone based developer suitable for X-ray films. The following results were obtained:

| Emulsion No. | Initial Fog | Log Speed | Incubation Fog |
|--------------|-------------|-----------|----------------|
| 1            | 0.15        | 5.35      | 0.15           |
| 2            | 0.17        | 5.50      | 0.65           |
| 3            | 0.15        | 5.42      | 0.25           |

(Incubation = 7 days at 125° F., 66 percent R.H.).

It will be noted that the inclusion of the polyethylene oxide afforded an increase in speed but an unacceptable increase in fog. This fog was reduced by the addition of the phenobarbitone almost to the level of the control emulsion.

(Phenidone is a Registered Trade Mark of Ilford Limited).

I claim as my invention:

- 45 1. In a process for the production of a gelatino silver halide emulsion which comprises forming the emulsion by a technique including a step wherein the emulsion is sulfur sensitized, and adding to the emulsion an ethylene oxide condensate sensitizer to increase the speed of the emulsion and the contrast of images developed therein, the improvement consisting of adding to the emulsion at least 1 g. per gram mole of silver halide present, of a compound of the formula:



wherein R<sub>1</sub> is an aryl group and R<sub>2</sub> is a lower alkyl group.

- 60 2. A process according to claim 1 wherein in the compound of the formula defined therein R<sub>1</sub> is phenyl and R<sub>2</sub> is ethyl.

- 65 3. A process according to claim 1 wherein the compound of the formula defined therein is added to the emulsion as an aqueous alkaline solution.

- 70 4. A process according to claim 1 wherein both the ethylene oxide condensate and the compound of the formula defined in claim 1 are added after the emulsion has been sulfur sensitized.

- 75 5. A sulfur-sensitized gelatino silver halide emulsion sensitized with an ethylene oxide condensate to increase the speed of the emulsion and the contrast of images developed therein, said emulsion including at least 1 g. per gram mole of silver halide present, of a compound of the formula:

3,617,290



**4**

wherein R<sub>1</sub> is an aryl group and R<sub>2</sub> is a lower alkyl group.

6. The emulsion of claim 5 wherein R<sub>1</sub> is phenyl and R<sub>2</sub> is ethyl.

\* \* \* \* \*

**5**

**10**

**15**

**20**

**25**

**30**

**35**

**40**

**45**

**50**

**55**

**60**

**65**

**70**

**75**